

Feb. 14, 1956

R. B. SNYDER

2,734,857

PROCESS OF COATING A CATHODE-HEATER ELEMENT

Filed Oct. 11, 1951

FIG. 1



FIG. 2



FIG. 3



INVENTOR:  
RUSSELL B. SNYDER  
BY  
*Francis W. Scotty*  
HIS ATTORNEY

1

2,734,857

**PROCESS OF COATING A CATHODE-HEATER ELEMENT**

Russell B. Snyder, Chicago, Ill., assignor to The Rauland Corporation, a corporation of Illinois

Application October 11, 1951, Serial No. 250,911

5

10

3 Claims. (Cl. 204—181)

This invention relates to cathode-heater elements for 15 electron-discharge devices and more particularly to insulated cathode-heater elements and to processes for forming the insulating coating on such elements.

In the fabrication of cathode-heater elements for indirectly-heated cathodes of electron-discharge devices, it 20 is necessary to provide some means of insulating the electron-emissive cathode element from its indirect-heater element. In accordance with common practice in the art, the heater element is provided with an insulating coating of refractory oxide prior to insertion in the cathode member. This insulating coating must be hard, adherent, and relatively tough to withstand all the processing operations and handling during the fabrication of the tube. Moreover, the coating must retain its insulating properties 25 at the high operating temperatures, usually in excess of 1000° C., of the heater element. The material most commonly used for the insulating coating is aluminum oxide, sometimes referred to as alumina or Alundum, having a minimum of impurities and of very fine particle size.

Insulating coatings of this type have been applied to 30 heater elements in numerous manners, as by spraying, drag coating, and the process generally referred to as cataphoretic coating. Subsequent to the application of the insulating material, the heater is fired in a hydrogen or non-oxidizing atmosphere at a temperature below the fusion point of the refractory oxide insulator. While the resultant coating is relatively tough and adherent, great care has been required in the subsequent handling to avoid undesirable flaking or peeling. Moreover, insulating coatings applied in accordance with known procedures are rather sensitive to vibration, and tubes employing heater elements having coatings of this type are 35 consequently susceptible to premature failure in certain applications.

It is an important object of the present invention to provide a new and improved cathode-heater element having an insulating coating which is tougher, harder, less brittle, and which better withstands vibration than those known heretofore.

It is a further object of the invention to provide a new and improved process for applying an insulating coating to a cathode-heater element.

In accordance with the invention, a new and improved process of forming an insulating coating on a cathode-heater element for an electron-discharge device comprises the steps of cataphoretically depositing on the heater element a coating comprising an electrically insulating refractory oxide, dipping the coated heater element in an alcohol solution of an organic silicate, and subsequently firing the coated heater element in a non-oxidizing atmosphere at a temperature above the fusing point of silica and below both the boiling point of silica and the boiling point of the refractory oxide.

The features of the present invention which are believed to be novel are set forth with particularity in the

2

appended claims. The invention, together with further objects and advantages thereof, may best be understood, however, by reference to the following description taken in connection with the accompanying drawing, in the several figures of which like reference numerals indicate like elements, and in which:

Figure 1 is a flow diagram or process chart of a new and improved method of forming an insulating coating in accordance with the present invention;

Figure 2 is a side elevation of a new and improved cathode-heater element constructed in accordance with the invention; and

Figure 3 is an enlarged cross-sectional view taken along the line 3—3 of Figure 2.

A cathode-heater element for an electron-discharge device may be provided with an insulating coating having the desired properties in accordance with the procedure set forth diagrammatically in Figure 1. The metallic base member, having a high resistivity and usually constructed either of tungsten or an alloy of tungsten and molybdenum, is first provided with a refractory oxide coating in a known manner. For example, the well known cataphoretic deposition process may be employed. In accordance with this process, fine particles of aluminum oxide are suspended in a suitable liquid medium such as water and methanol containing small amounts of hydrated aluminum nitrate and hydrated magnesium nitrate. A unidirectional potential difference, which may be of the order of 100 volts, is applied between the heater element to be coated and another electrode which are immersed in the coating suspension. In the presence of the applied potential difference, the aluminum nitrate hydrolyses to aluminum hydroxide and nitric acid, and the aluminum hydroxide is cataphorized or caused to migrate to the heater element. In the process, particles of alumina are trapped on the surface of the heater element by the aluminum hydroxide which acts as a temporary binder.

When the coating thus deposited has built up to the desired thickness, the heater element is removed from the coating suspension and dried in air for about one-half hour at room temperature to permit the coating to set on the base metal. At this stage in the process, the coated heater element is in precisely the same condition as those produced by conventional methods immediately prior to the hydrogen firing operation.

In accordance with the present invention, the heater element bearing the cataphorized insulating coating of alumina is dipped in a non-aqueous silica solution, such as a solution of ethyl ortho-silicate or other alkyl ester of silicic acid in an alcohol solvent. Alternatively, the non-aqueous silica solution may be applied by spraying or in any other equivalent manner. The amount of non-aqueous silica solution thus applied is not critical; in practice, the coated heater element is preferably immersed in the silica solution and immediately withdrawn, it being only necessary to moisten the refractory oxide coating. The moistened coating is then permitted to dry in air at room temperature for about one-half hour. Hydrolysis of the silica solution and subsequent evaporation of the solvent leaves substantially pure silica finely dispersed throughout the particles of refractory oxide.

At this stage of the procedure, either of two courses may be pursued. According to one alternative, the heater element may be directly fired in a non-oxidizing atmosphere, such as hydrogen, an inert gas, or in a vacuum, at a temperature above the fusing point of silica (about 1710° C.) and below both the boiling point of silica and the boiling point of the refractory oxide employed. By the firing operation, the silica is fused to serve as a binder for the insulating coating. The firing

operation may be accomplished with the aid of a radio-frequency induction heating field if desired.

According to the other alternative, following the application of the non-aqueous silica solution, the coated heater element is baked in air for about 30 minutes at an elevated temperature below the fusing point of silica, for example about 400° C. Following this baking operation the coating is sufficiently hard and tough to withstand ordinary handling and insertion into the cathode sleeve during the assembly of the electron-discharge device. Moreover, removal of certain portions of the coating at the terminals of the heater element to permit electrical connection of the leads thereto may be accomplished much more readily prior to the fusion of the silica bond than afterwards. The heater element may be fired in a non-oxidizing atmosphere, as described above, at any subsequent stage in the assembly operation or the firing operation may be omitted entirely in which case the fusion of the silica binder is accomplished during the initial operation of the completed tube by passage of heater current.

While the process has been described in connection with the use of pulverulent Alundum or aluminum oxide, other refractory oxides may be employed as the insulating material. The refractory oxides comprise, in addition to alumina, the oxides of zirconium, beryllium, thorium, and magnesium which are known respectively as zirconia, beryllia, thoria, and magnesia. Certain of these oxides are not readily adaptable to cataphoretic deposition, but other well known processes such as drag coating and spraying may be employed to apply the insulating material to the base metal. In the event that one of these latter processes is employed, the refractory oxide may be suspended in the non-aqueous silica solution so that both are applied simultaneously, or the ethyl ortho-silicate or other non-aqueous silica solution may be applied after formation of the refractory oxide coating.

Forming of the heater element may be accomplished at any stage in the process prior to the firing operation, although this may most readily be accomplished prior to the commencement of the coating process.

The significance of the particle size of the refractory oxide is well known in the art. In general, it is essential that the refractory oxide be pulverulent in the form of discrete particles of 50 microns or less in diameter, an average particle size of 10 to 20 microns being most satisfactory. Coarse particles usually result in soft coatings which are apt to yield slightly and separate when the wire is bent in forming or handling. On the other hand, fine particles result in hard brittle coatings which often rupture if the wire is sharply bent.

A cathode-heater element constructed in accordance with the present invention is illustrated in Figures 2 and 3 and comprises a metallic base member 10 of tungsten or tungsten-molybdenum alloy, coated with a thin layer 11 of refractory oxide bonded with fused silica.

The invention is applicable to all types of cathode-heater elements, regardless of the physical configuration and the type of ultimate apparatus in which the heater is to be employed. Specifically, heater elements of various forms coated in accordance with the invention may

be employed in high-vacuum receiving tubes, cathode-ray tubes, gas filled tubes such as thyratrons and the like, and special purpose tubes. The coating is tough, hard and durable and may be inserted into the cathode proper with little or no risk of damage. In the completed apparatus, the risk of failure caused by damage to the coating from even the most extreme vibration is substantially obviated.

While the process has been described as employing a single refractory oxide, it is apparent that the insulating material may comprise two or more of the refractory oxides if desired. Consequently, the term "refractory oxide" is employed in the appended claims in both the singular and plural sense.

While particular embodiments of the present invention have been shown and described, it is apparent that various changes and modifications may be made, and it is therefore contemplated in the appended claims to cover all such changes and modifications as fall within the true spirit and scope of the invention.

I claim:

1. The process of forming an insulating coating on a cathode-heater element for an electron-discharge device which comprises the steps of: cataphoretically depositing on said heater element an electrically insulating refractory oxide coating; dipping said coated heater element in an alcohol solution of an organic silicate; and subsequently firing said coated heater element in a non-oxidizing atmosphere at a temperature above the fusing point of silica and below both the boiling point of silica and the boiling point of said refractory oxide.

2. The process of forming an insulating coating on a cathode-heater element for an electron-discharge device which comprises the steps of: cataphoretically depositing on said heater element an electrically insulating refractory oxide coating; dipping said coated heater element in a solution of ethyl ortho-silicate in an alcohol solvent; and subsequently firing said coated heater element in a non-oxidizing atmosphere at a temperature above the fusing point of silica and below both the boiling point of silica and the boiling point of said refractory oxide.

3. The process of forming an insulating coating on a cathode-heater element for an electron-discharge device which comprises the steps of: cataphoretically depositing on said heater element an aluminum oxide coating; drying said coated heater element; dipping said coated heater element in a solution of ethyl ortho-silicate in an alcohol solvent; drying said heater element; and subsequently firing said coated heater element in a non-oxidizing atmosphere at a temperature above the fusing point of silica and below both the boiling point of silica and the boiling point of said aluminum oxide.

#### References Cited in the file of this patent

#### UNITED STATES PATENTS

|           |           |                |
|-----------|-----------|----------------|
| 1,874,542 | Kaul      | Aug. 30, 1932  |
| 1,926,407 | Ruben     | Sept. 12, 1933 |
| 2,158,665 | O'Neill   | May 16, 1939   |
| 2,307,018 | Cardell   | Jan. 5, 1943   |
| 2,348,045 | Wooten    | May 2, 1944    |
| 2,552,535 | De Santis | May 15, 1951   |